

# United States Patent

[19]

[11] 3,895,090

Kobayashi et al.

[45] July 15, 1975

[54] **METHOD FOR DIRECT SPINNING OF POLYETHYLENE-1,2-DIPHENOXYETHANE-P,P'-DICARBOXYLATE FIBERS**

[75] Inventors: **Hidehiko Kobayashi**, Tokyo; **Masatsugu Yoshino**, Saitamaken; **Kazuya Neki**, Saitamaken, all of Japan

[73] Assignee: **Asahi Kasei Kogyo Kabushiki Kaisha**, Osaka, Japan

[22] Filed: **Mar. 26, 1969**

[21] Appl. No.: **810,775**

[30] **Foreign Application Priority Data**

Apr. 9, 1968 Japan..... 43-23061

[52] U.S. Cl..... **264/176 F**; **260/47 C**; **264/210 F**

[51] Int. Cl.<sup>2</sup>..... **D01D 5/08**

[58] Field of Search..... **264/210, 290, 176; 260/47 C, 75 R**

[56] **References Cited**

UNITED STATES PATENTS

- |           |         |                |       |           |
|-----------|---------|----------------|-------|-----------|
| 2,604,667 | 7/1952  | Hebeler        | ..... | 264/168   |
| 2,604,689 | 7/1952  | Hebeler        | ..... | 264/168   |
| 2,957,747 | 10/1960 | Bowling        | ..... | 264/210 F |
| 3,048,467 | 8/1962  | Roberts et al. | ..... | 264/210 F |
| 3,161,710 | 12/1964 | Turner         | ..... | 264/236   |

|           |         |                       |           |
|-----------|---------|-----------------------|-----------|
| 3,215,486 | 11/1965 | Hada et al. ....      | 264/210 F |
| 3,361,859 | 1/1968  | Cenzato.....          | 264/210 F |
| 3,475,381 | 10/1969 | Price et al. ....     | 260/75    |
| 3,513,110 | 5/1970  | Noether.....          | 264/290   |
| 3,624,031 | 11/1971 | Kobayashi et al. .... | 260/47 C  |
| 3,642,697 | 2/1972  | Kobayashi et al. .... | 260/47 C  |
| 3,654,225 | 4/1972  | Kobayashi et al. .... | 260/47 C  |

FOREIGN PATENTS OR APPLICATIONS

|           |         |                     |           |
|-----------|---------|---------------------|-----------|
| 131,320   | 11/1946 | Australia.....      | 260/47 C  |
| 1,046,069 | 10/1966 | United Kingdom..... | 260/47 C  |
| 1,047,978 | 11/1966 | United Kingdom..... | 264/290 T |
| 567,106   | 12/1958 | Canada.....         | 264/75    |

Primary Examiner—Jay H. Woo  
Attorney, Agent, or Firm—Fred Philpitt

[57]

**ABSTRACT**

Commercially useful polyethylene-1,2-diphenoxymethane-p,p'-dicarboxylate fibers are obtained by the direct spinning of a melt of polyethylene-1,2-diphenoxymethane-p,p'-dicarboxylate with a commercially feasible take-up speed of 1800–3500 m/min by maintaining an intrinsic viscosity and a residual carboxyl group of said polymer within the range of 0.4–1.3 and less than 20 equivalents/10<sup>6</sup> g., respectively, and when the monofilament denier is as thin as 1.5–0.3, the take-up speed can be reduced to a value of 1000–1800 m/min.

**5 Claims, No Drawings**

**METHOD FOR DIRECT SPINNING OF  
POLYETHYLENE-1,2-DIPHENOXYETHANE-P,P'-  
DICARBOXYLATE FIBERS**

In the production of fibers from a linear high molecular weight polymer which is spinnable by a melt-spinning process, it has been common heretofore to rely on a process which comprises stretching non-stretched fiber filaments having low tenacity, high elongation, low crystallinity and poor orientation to improve their crystallinity and orientation. Namely, it has required the two steps of (a) spinning and (b) stretching in the production.

It is not desirable to have two steps in the fiber formation from the standpoint of labor, equipment, apparatus, and production capacity.

For the production of useful fibers having high tenacity and low elongation only by the step of spinning, it is necessary to provide crystallinity and orientation sufficient as fibers to the fiber filaments spun during their travel from a spinneret to a take-up point. Attempts to take up extruded fiber filaments at such high velocities, such as more than 5200 yd./min., and 3000-5200 yd./min. have been proposed in U.S. Pat. No. 2,604,667 and 2,604,689, respectively.

However, such high speed taking up as above-mentioned, not only is accompanied by mechanical difficulties and danger but also the fiber filaments taken up at such high velocities have relatively large residual elongation and low yield strength. On this account, resultant fiber filaments bring about many difficult points when used practically in subsequent steps of processing such as the problems encountered in the steps of weaving, processings and treatment thereof and the problem of non-uniformity of woven products.

Accordingly, it is an object of the present invention to provide a method for directly spinning polyethylene-1,2-diphenoxymethane-p,p'-dicarboxylate fibers which permits one to overcome the above-mentioned drawbacks of conventional direct spinning methods.

Other objects and advantages will be apparent from the description which hereinafter follows. It has been discovered by the inventors of the present application that fibers having extremely useful properties can be obtained from polyethylene-1,2-diphenoxymethane-p,p'-dicarboxylate which satisfies specified conditions by taking up the filaments at a velocity much lower than that expectable from conventional way of thinking.

Namely the present invention consists in a novel direct spinning method of polyethylene-1,2-diphenoxymethane-p,p'-dicarboxylate fibers which comprises taking up the filament yarns spun with a common spinning machine from polyethylene-1,2-diphenoxymethane-p,p'-dicarboxylate which satisfies specified conditions.

The polymers used in the practice of the present invention must be a polyethylene-1,2-diphenoxymethane-p,p'-dicarboxylate containing at least 70 mol.% of repetition unit of



whose intrinsic viscosity  $[\eta]$  of polymer is more than 0.4 and less than 1.3, (inclusive) and containing less than 20 eq./ $10^6$  g. (inclusive) of residual carboxyl group in the polymer.

5 An intrinsic viscosity  $[\eta]$  of the polymer less than 0.4 and more than 1.3, is not preferable because breakage of filaments frequently occurs in such cases.

When the amount of residual carboxyl radical in the polymer is more than 20 eq./ $10^6$  g. and the filaments 10 are taken up at such a low speed as above-mentioned, only filaments having low yield strength can be obtained. On the other hand when it is less than 20 eq./ $10^6$  g. superior fibers having a high yield strength can be obtained even when filament yarns are taken up at a

15 relatively low take-up speed. Further the spinnability at the time of actual spinning is exceedingly superior and the fibers having very high stability can be obtained at a spinning temperature ranging from 255° to 320°C with a high production efficiency even in case of a high speed take-up, regardless to say, in case of relatively low speed take-up.

The intrinsic viscosities  $[\eta]$  herein referred to, are values as measured in a solvent consisting of a 2:1 mixture by weight of tetrachloroethene and phenol at 25 35°C.

The residual carboxyl radicals herein referred to, are values measured by a method which resorts to titration with a solution of caustic soda and benzyl alcohol by 30 using, as a solvent, benzyl alcohol, and, as an indicator, phenol red. [See H. H. Pohl (Annal. Chem., 26, 1614 (1954)).]

The yield strengths herein referred to, are values determined from stress-strain curves in case where samples 35 20 cm long are stretched at an elongation speed of 100% per minute.

When samples do not show clear yield point, they are determined as an intercepting point of two lines extrapolated from both low elongation side and high elongation side.

40 The above-mentioned polymer can be produced by subjecting 1,2-bis-(paracarbomethoxy)-phenoxyethane or its ester-forming derivatives and ethylene glycol to ester-exchange reaction in the presence 45 of a catalyst to form bisglycol of 1,2-bis-(paracarbomethoxy)-phenoxyethane and then subjecting the latter to condensation polymerization in the presence of a polymerization catalyst, at an elevated temperature and under a reduced pressure while eliminating excessive glycol produced in the condensation.

50 In the production of the above-mentioned polyester ether, it may be possible to add a small amount of one or more comonomers, i.e. one or more of the substances selected from glycols other than ethylene glycol, dicarboxylic acids and hydroxycarboxylic acids. 55 Thus the constitution material suitable to the method of the present invention and consisting essentially of polyethylene-1,2-diphenoxymethane-p,p'-dicarboxylate may contain up to 30 mol % of another glycol such as diethylene glycol, tetramethylene glycol, hexamethylene glycol or the like. Further, the molecule may contain up to 30 mol % of another acid. Illustrative copolymerizable acids suitable to the present method include hexahydroterephthalic acid, terephthalic acid, isophthalic acid, bibenzoic acid, adipic acid, sebacic acid, azelaic acid, naphthalic acid, 2,5-dimethyl terephthalic acid.

These third component may be added during the polymerization step, or before the reaction together with initial starting materials. Alternatively, it is also possible to polymerize it separately and mixed with polyethylene-1,2-diphenoxoethane-p,p'-dicarboxylate by melting.

In the practice of the method of the present invention, fibers having a yield strength of more than 1.0 g/d, an initial modulus of elasticity of more than 70 g/d, a breaking strength of more than 3.0 g/d and a residual elongation of less than 80% can be obtained by taking up the fiber filaments produced by melt-extrusion at a speed of more than 1800 m/min. but a take-up speed greater than 3500 m/min. is not preferable because it brings about frequent breakages of filaments.

According to the method of the present invention which is characterized in taking up filaments at a relatively low speed, it is surprising enough that the lower limit of taking-up can be reduced nearly down to a common spinning speed in the spinning of fine filaments. Namely, in case monofilament denier is in the range of less than 0.5 and greater than 0.2 (inclusive), it is possible to produce fibers having a large tenacity and useful in the practical use even at a take-up speed of 1000 m/min and in case monofilament denier is about 1.0 d, it is possible to produce fibers having a large tenacity and useful in the practical use even at a take-up speed of 1500 m/min.

Application of a common production method of synthetic fibers consisting of two steps of spinning and stretching, to such ultrafine filaments as above-mentioned, is difficult because of various problems such as breakage of yarns or monofilaments and development of fluff but application of the direct spinning method according to the present invention has made the production of ultrafine filaments possible with exceedingly high efficiency. However, application in case of less than 0.2 denier is not preferable on account of increase of breakage of monofilaments.

As above-mentioned, the fibers obtained in the method of the present invention have properties superior to those of the filaments obtained by a conventional direct spinning method but it is possible to provide a production method of practically very useful fibers furnished with even much more superior properties if considerations are given to various conditions such as those regarding the polymer, spinneret, the temperature of atmosphere surrounding the course of extruded filaments upto a take-up point, method for taking up filaments and proper limitations thereof. Description will be directed firstly to the condition regarding the polymer.

Any known combination of ester-exchange catalyst and polymerization catalyst useful in the production of polymer can be utilized so long as residual carboxyl radical in the polymer becomes less than 20 eq./10<sup>6</sup> g. (inclusive) by the proper selection of other polymerization conditions such as polymerization time and temperature but when a combination system consisting of a specified ester exchange catalyst and polymerization catalyst is used in the production of polymer, and fibers are produced therefrom by a high speed spinning process, resultant fibers have particularly excellent properties such as greater yield strength, greater breaking strength, lower residual elongation, etc.. As preferable combinations of ester exchange catalyst and polymerization catalyst, combinations of a barium compound

and a tin compound; a barium compound and an antimony compound; a calcium compound and an antimony compound; are illustrated.

Useful compounds for ester exchange catalyst include elementary metal, carbonate, oxide, hydroxide, acetate and borate of barium or calcium.

As antimony compounds useful for polymerization catalyst, salts of antimony with inorganic or organic acid, double salts such as potassium, antimony tartrate 10 salts of antimonate acid, (e.g. ammonium pyroantimonate), oxides, glucoside, catechol complex salts, etc. are illustrated.

As tin compounds, organic tin compounds expressed by a general formula of  $R_mSnX_{4-m}$  are suitable.

15 [wherein Sn is tin atom, m is an integer of 1-4, Vx is a valency of X atom, 4-m/vx is an integer of 0-3, R is an aliphatic group having 1-18 carbon atoms, a cyclic radical having 3-6 rings, or an aromatic group, and X is  $-R$ ,  $-OR$ ,  $-OH$ ,  $-SnR_3$ ,

20

halogen,  $-O-$ , or

25



halogen,  $-O-$ , or

25



30 (wherein R has same meaning as above-defined, and R' is a divalent R having the above-defined meaning)].

The above-mentioned ester-exchange catalyst is used in an amount of 0.005-0.5% (inclusive) by weight, preferably 0.01-0.3% (inclusive) by weight relative to the produced polymer. The above-mentioned polymerization catalyst is used in an amount of 0.005-0.5% (inclusive) by weight, preferably 0.01-0.5% (inclusive) by weight relative to the produced polymer.

35 The addition of a phosphor compound such as triphenyl phosphite, phosphoric acid, phosphorous acid, as a stabilizer for coloring, and TiO<sub>2</sub> as a delustering agent, is not harmful to the effectiveness of the present invention.

40 When the catalyst system consisting of the above-mentioned specified combination is used in the production of polymer, the crystallization velocity of the resultant polymer is particularly fast. Half crystallization time as measured by changing the temperature of polymers melted at 290°C for 10 minutes immediately to 220°C and maintaining the polymers at this temperature by using a Differential Scanning Calorimeter made by Perkin Elmer Co., is within 2 minutes. This fast crystallization velocity is believed to give advantageous influence upon stretching, orientation and crystallization at the time of high speed taking-up.

45 50 55 It is really surprising that such a small amount of catalyst system gives advantageous influence upon the properties of fibers and usefulness of the method of the present invention can be highly evaluated.

60 Description will be directed secondly to the condition regarding spinneret. It is preferable that the hole diameter of spinneret used in the spinning of the present invention is greater than 0.25 mmφ and smaller than 0.9 mmφ (inclusive). When it is within this range, the stability is extremely good at the time of spinning. 65 When the hole length of spinneret is greater than 1.5 mm and smaller than 10 mm (inclusive), most uniform fibers can be obtained. When it is smaller than 1.5 mm,

the non-uniformity tends to appear in the physical properties of fibers due to non-uniform flow of melted material. There is no need of the hole length being longer than 10 mm.

Description will be directed thirdly to the condition of the atmosphere. It is preferable to make extruded filament yarns pass through a hot atmosphere maintained at 10°C – 180°C over the range of distance from the spinneret longer than 30 cm and shorter than 2 m before taking-up. It is not preferable to extrude melted material in a cold atmosphere of lower than 10°C or to do extrusion in the state that gas or spray of liquid cooled below 10°C is being blown to a spinneret because the yield strength of fibers is reduced. It is also a condition which lowers the orientation of molecular chain of filament yarns and affords products inferior in physical properties to make filaments pass in a hot atmosphere higher than 180°C. It is neither preferable to adopt a heating range shorter than 30 cm, nor a longer range than 2 m. In the control of hot atmosphere, beside the control of cooling speed by way of dried hot wind which has been conventionally used in the spinning of polyester-type fibers, the use of hot wind wetted upto higher than 65% RH makes the control easier and affords better result.

Description will be directed fourthly to taking-up method. The term "take-up" herein used is a device which determines the running speed of extruded filament yarns after cooled and solidified. It is not limited only to a device for winding up filament yarns on bobbins which are used together with a common driving mechanism. It also includes the entire apparatus containing a device which runs the filament yarns at a substantially high speed such as an air jet device, etc.

In the practice of the present invention, if one or more of a material which affords friction to the filaments yarns is inserted between the part from a spinneret and a take-up point and the filaments yarns are rubbed while passing therethrough, it is possible to achieve the effectiveness close to that of high speed cases by a take-up speed lying in a relatively low range and also possible to prevent the unevenness of denier which is produced by the direct transmission of fluctuation of tension at a take-up part to a spinneret.

The material which affords friction comprises a pin which does not rotate or a revolving roller. When a revolving material is used, it is necessary to make the peripheral speed of revolving material slower or faster than the speed of filament yarns.

If such a treatment is given to the surface of the friction-affording material that the friction with the filament yarns is increased, greater effectiveness can be attained.

Based upon the above-mentioned factors which make the method of the present invention advantageous, it is possible to obtain more beneficent result by combining two or more of the factors.

The present invention may be more fully understood from the following examples which are offered by way of illustration and not by way of limitation. All parts and per cent are by weight.

## EXAMPLE 1

Polyethylene-1,2-diphenoxymethane-p,p'-dicarboxylate having an intrinsic viscosity of polymer of 0.65 and an amount of residual carboxyl group of polymer of 16 eq./10<sup>6</sup> g., produced by the polymerization using 0.03 part of manganese acetate as an ester exchange catalyst and 0.01 part of germanium dioxide as a polymerization catalyst, was extruded through a spinneret having a diameter of each hole of 0.35 mmφ and a length of 2 mm at a spinning temperature of 290°C and subjected to spinning under varied spinning conditions. Results obtained are indicated in Table I.

Table I

| Take up speed (m/min.) | Fineness (denier) | Yield strength (g/d) | Tenacity at break (g/d) | Elongation at break (%) | Initial elastic modulus (g/d) |
|------------------------|-------------------|----------------------|-------------------------|-------------------------|-------------------------------|
| 1600                   | 1.9               | 0.75                 | 2.7                     | 110                     | 54.4                          |
| 1800                   | 2.0               | 1.1                  | 3.1                     | 80                      | 78.0                          |
| 1800                   | 3.3               | 1.05                 | 3.0                     | 90                      | 73.0                          |
| 2500                   | 0.8               | 1.4                  | 3.7                     | 51                      | 110.0                         |
| 2500                   | 2.1               | 1.2                  | 3.5                     | 57                      | 100.2                         |
| 2500                   | 5.2               | 1.0                  | 3.2                     | 63                      | 93.0                          |
| 3000                   | 1.8               | 1.8                  | 3.6                     | 50                      | 111.0                         |
| 3000                   | 3.3               | 1.5                  | 3.3                     | 54                      | 101.0                         |
| 3500                   | 2.3               | 2.8                  | 4.2                     | 45                      | 153.2                         |
| 3500                   | 3.1               | 2.4                  | 3.8                     | 47                      | 109.8                         |
| 3500                   | 5.0               | 2.0                  | 3.5                     | 54                      | 105.0                         |

## COMPARATIVE EXAMPLE 1

Polyethylene-1,2-diphenoxymethane-p,p'-dicarboxylate having an intrinsic viscosity of 0.61 and a residual carboxyl radical of polymer of 33 eq./10<sup>6</sup> g., produced by the polymerization using 0.03 parts of manganese acetate as an ester exchange catalyst and 0.01 part of germanium dioxide as a polymerization catalyst, was extruded from a spinneret having a diameter of each hole of 0.35 mmφ and a length of 2 mm at a spinning temperature of 285°C. The properties of fibers obtained under various spinning conditions, are shown in the following Table II.

Table II

| Take-up speed (m/min.) | Fineness (denier) | Yield strength (g/d) | Tenacity at break (g/d) | Elongation at break (%) | Initial elastic modulus (g/d) |
|------------------------|-------------------|----------------------|-------------------------|-------------------------|-------------------------------|
| 1600                   | 2.0               | 0.53                 | 2.6                     | 119                     | 53.3                          |
| 1800                   | 2.3               | 0.69                 | 2.9                     | 92                      | 75.0                          |
| 1800                   | 3.0               | 0.51                 | 2.7                     | 99                      | 61.0                          |
| 2500                   | 1.0               | 1.0                  | 3.3                     | 60                      | 105.0                         |
| 2500                   | 1.9               | 0.77                 | 3.1                     | 64                      | 93.3                          |
| 2500                   | 5.1               | 0.69                 | 2.9                     | 80                      | 80.1                          |
| 3000                   | 2.2               | 1.2                  | 3.5                     | 53                      | 109.4                         |
| 3000                   | 3.3               | 1.0                  | 3.3                     | 57                      | 98.6                          |
| 3500                   | 2.0               | 2.6                  | 4.0                     | 47                      | 118.2                         |
| 3500                   | 3.4               | 2.1                  | 3.4                     | 49                      | 105.5                         |
| 3500                   | 5.2               | 2.0                  | 3.4                     | 56                      | 100.1                         |

## EXAMPLE 2

To 90 parts of 1,2-bis-(paracarboxymethoxy)-phenoxyethane, 75 parts of ethylene glycol, 0.01 part of calcium acetate as an ester-exchange catalyst were admixed and resultant mixture was heated at 220°C for

4 hours and formed methanol was eliminated. Thereafter, 10 parts of adipic acid, 0.01 part of antimony trioxide, 0.01 part of  $TiO_2$  and as a stabilizer, 0.1 part of triphenyl phosphite were charged in a polymerization vessel, and heated at 280°C under a reduced pressure of lower than 0.1 mm Hg while eliminating formed ethylene glycol. The intrinsic viscosity and the residual carboxyl group of the polymer were 0.84 and 13 eq./10<sup>6</sup> g., respectively. Resultant polymer was extruded from a spinneret having a diameter of each hole of 0.45 mm, a length of each hole of 2 mm and number of holes of 24 at a spinning temperature of 300°C at an extrusion rate of 12 g./min. and resultant fibers were taken up at a speed of 2500 m/min. whereby excellent fibers having a tenacity of 3.6 g/d, elongation of 38%, initial modulus of elasticity of 114 g/d, and yield strength of 1.3 g/d were obtained.

### EXAMPLE 3

Polyethylene-1,2-diphenoxy ethane-<sup>20</sup> <sup>25</sup> <sup>30</sup> <sup>35</sup> <sup>40</sup> <sup>45</sup> <sup>50</sup> <sup>55</sup> <sup>60</sup> <sup>65</sup> <sup>70</sup> <sup>75</sup> <sup>80</sup> <sup>85</sup> <sup>90</sup> <sup>95</sup> <sup>100</sup> <sup>105</sup> <sup>110</sup> <sup>115</sup> <sup>120</sup> <sup>125</sup> <sup>130</sup> <sup>135</sup> <sup>140</sup> <sup>145</sup> <sup>150</sup> <sup>155</sup> <sup>160</sup> <sup>165</sup> <sup>170</sup> <sup>175</sup> <sup>180</sup> <sup>185</sup> <sup>190</sup> <sup>195</sup> <sup>200</sup> <sup>205</sup> <sup>210</sup> <sup>215</sup> <sup>220</sup> <sup>225</sup> <sup>230</sup> <sup>235</sup> <sup>240</sup> <sup>245</sup> <sup>250</sup> <sup>255</sup> <sup>260</sup> <sup>265</sup> <sup>270</sup> <sup>275</sup> <sup>280</sup> <sup>285</sup> <sup>290</sup> <sup>295</sup> <sup>300</sup> <sup>305</sup> <sup>310</sup> <sup>315</sup> <sup>320</sup> <sup>325</sup> <sup>330</sup> <sup>335</sup> <sup>340</sup> <sup>345</sup> <sup>350</sup> <sup>355</sup> <sup>360</sup> <sup>365</sup> <sup>370</sup> <sup>375</sup> <sup>380</sup> <sup>385</sup> <sup>390</sup> <sup>395</sup> <sup>400</sup> <sup>405</sup> <sup>410</sup> <sup>415</sup> <sup>420</sup> <sup>425</sup> <sup>430</sup> <sup>435</sup> <sup>440</sup> <sup>445</sup> <sup>450</sup> <sup>455</sup> <sup>460</sup> <sup>465</sup> <sup>470</sup> <sup>475</sup> <sup>480</sup> <sup>485</sup> <sup>490</sup> <sup>495</sup> <sup>500</sup> <sup>505</sup> <sup>510</sup> <sup>515</sup> <sup>520</sup> <sup>525</sup> <sup>530</sup> <sup>535</sup> <sup>540</sup> <sup>545</sup> <sup>550</sup> <sup>555</sup> <sup>560</sup> <sup>565</sup> <sup>570</sup> <sup>575</sup> <sup>580</sup> <sup>585</sup> <sup>590</sup> <sup>595</sup> <sup>600</sup> <sup>605</sup> <sup>610</sup> <sup>615</sup> <sup>620</sup> <sup>625</sup> <sup>630</sup> <sup>635</sup> <sup>640</sup> <sup>645</sup> <sup>650</sup> <sup>655</sup> <sup>660</sup> <sup>665</sup> <sup>670</sup> <sup>675</sup> <sup>680</sup> <sup>685</sup> <sup>690</sup> <sup>695</sup> <sup>700</sup> <sup>705</sup> <sup>710</sup> <sup>715</sup> <sup>720</sup> <sup>725</sup> <sup>730</sup> <sup>735</sup> <sup>740</sup> <sup>745</sup> <sup>750</sup> <sup>755</sup> <sup>760</sup> <sup>765</sup> <sup>770</sup> <sup>775</sup> <sup>780</sup> <sup>785</sup> <sup>790</sup> <sup>795</sup> <sup>800</sup> <sup>805</sup> <sup>810</sup> <sup>815</sup> <sup>820</sup> <sup>825</sup> <sup>830</sup> <sup>835</sup> <sup>840</sup> <sup>845</sup> <sup>850</sup> <sup>855</sup> <sup>860</sup> <sup>865</sup> <sup>870</sup> <sup>875</sup> <sup>880</sup> <sup>885</sup> <sup>890</sup> <sup>895</sup> <sup>900</sup> <sup>905</sup> <sup>910</sup> <sup>915</sup> <sup>920</sup> <sup>925</sup> <sup>930</sup> <sup>935</sup> <sup>940</sup> <sup>945</sup> <sup>950</sup> <sup>955</sup> <sup>960</sup> <sup>965</sup> <sup>970</sup> <sup>975</sup> <sup>980</sup> <sup>985</sup> <sup>990</sup> <sup>995</sup> <sup>1000</sup> <sup>1005</sup> <sup>1010</sup> <sup>1015</sup> <sup>1020</sup> <sup>1025</sup> <sup>1030</sup> <sup>1035</sup> <sup>1040</sup> <sup>1045</sup> <sup>1050</sup> <sup>1055</sup> <sup>1060</sup> <sup>1065</sup> <sup>1070</sup> <sup>1075</sup> <sup>1080</sup> <sup>1085</sup> <sup>1090</sup> <sup>1095</sup> <sup>1100</sup> <sup>1105</sup> <sup>1110</sup> <sup>1115</sup> <sup>1120</sup> <sup>1125</sup> <sup>1130</sup> <sup>1135</sup> <sup>1140</sup> <sup>1145</sup> <sup>1150</sup> <sup>1155</sup> <sup>1160</sup> <sup>1165</sup> <sup>1170</sup> <sup>1175</sup> <sup>1180</sup> <sup>1185</sup> <sup>1190</sup> <sup>1195</sup> <sup>1200</sup> <sup>1205</sup> <sup>1210</sup> <sup>1215</sup> <sup>1220</sup> <sup>1225</sup> <sup>1230</sup> <sup>1235</sup> <sup>1240</sup> <sup>1245</sup> <sup>1250</sup> <sup>1255</sup> <sup>1260</sup> <sup>1265</sup> <sup>1270</sup> <sup>1275</sup> <sup>1280</sup> <sup>1285</sup> <sup>1290</sup> <sup>1295</sup> <sup>1300</sup> <sup>1305</sup> <sup>1310</sup> <sup>1315</sup> <sup>1320</sup> <sup>1325</sup> <sup>1330</sup> <sup>1335</sup> <sup>1340</sup> <sup>1345</sup> <sup>1350</sup> <sup>1355</sup> <sup>1360</sup> <sup>1365</sup> <sup>1370</sup> <sup>1375</sup> <sup>1380</sup> <sup>1385</sup> <sup>1390</sup> <sup>1395</sup> <sup>1400</sup> <sup>1405</sup> <sup>1410</sup> <sup>1415</sup> <sup>1420</sup> <sup>1425</sup> <sup>1430</sup> <sup>1435</sup> <sup>1440</sup> <sup>1445</sup> <sup>1450</sup> <sup>1455</sup> <sup>1460</sup> <sup>1465</sup> <sup>1470</sup> <sup>1475</sup> <sup>1480</sup> <sup>1485</sup> <sup>1490</sup> <sup>1495</sup> <sup>1500</sup> <sup>1505</sup> <sup>1510</sup> <sup>1515</sup> <sup>1520</sup> <sup>1525</sup> <sup>1530</sup> <sup>1535</sup> <sup>1540</sup> <sup>1545</sup> <sup>1550</sup> <sup>1555</sup> <sup>1560</sup> <sup>1565</sup> <sup>1570</sup> <sup>1575</sup> <sup>1580</sup> <sup>1585</sup> <sup>1590</sup> <sup>1595</sup> <sup>1600</sup> <sup>1605</sup> <sup>1610</sup> <sup>1615</sup> <sup>1620</sup> <sup>1625</sup> <sup>1630</sup> <sup>1635</sup> <sup>1640</sup> <sup>1645</sup> <sup>1650</sup> <sup>1655</sup> <sup>1660</sup> <sup>1665</sup> <sup>1670</sup> <sup>1675</sup> <sup>1680</sup> <sup>1685</sup> <sup>1690</sup> <sup>1695</sup> <sup>1700</sup> <sup>1705</sup> <sup>1710</sup> <sup>1715</sup> <sup>1720</sup> <sup>1725</sup> <sup>1730</sup> <sup>1735</sup> <sup>1740</sup> <sup>1745</sup> <sup>1750</sup> <sup>1755</sup> <sup>1760</sup> <sup>1765</sup> <sup>1770</sup> <sup>1775</sup> <sup>1780</sup> <sup>1785</sup> <sup>1790</sup> <sup>1795</sup> <sup>1800</sup> <sup>1805</sup> <sup>1810</sup> <sup>1815</sup> <sup>1820</sup> <sup>1825</sup> <sup>1830</sup> <sup>1835</sup> <sup>1840</sup> <sup>1845</sup> <sup>1850</sup> <sup>1855</sup> <sup>1860</sup> <sup>1865</sup> <sup>1870</sup> <sup>1875</sup> <sup>1880</sup> <sup>1885</sup> <sup>1890</sup> <sup>1895</sup> <sup>1900</sup> <sup>1905</sup> <sup>1910</sup> <sup>1915</sup> <sup>1920</sup> <sup>1925</sup> <sup>1930</sup> <sup>1935</sup> <sup>1940</sup> <sup>1945</sup> <sup>1950</sup> <sup>1955</sup> <sup>1960</sup> <sup>1965</sup> <sup>1970</sup> <sup>1975</sup> <sup>1980</sup> <sup>1985</sup> <sup>1990</sup> <sup>1995</sup> <sup>2000</sup> <sup>2005</sup> <sup>2010</sup> <sup>2015</sup> <sup>2020</sup> <sup>2025</sup> <sup>2030</sup> <sup>2035</sup> <sup>2040</sup> <sup>2045</sup> <sup>2050</sup> <sup>2055</sup> <sup>2060</sup> <sup>2065</sup> <sup>2070</sup> <sup>2075</sup> <sup>2080</sup> <sup>2085</sup> <sup>2090</sup> <sup>2095</sup> <sup>2100</sup> <sup>2105</sup> <sup>2110</sup> <sup>2115</sup> <sup>2120</sup> <sup>2125</sup> <sup>2130</sup> <sup>2135</sup> <sup>2140</sup> <sup>2145</sup> <sup>2150</sup> <sup>2155</sup> <sup>2160</sup> <sup>2165</sup> <sup>2170</sup> <sup>2175</sup> <sup>2180</sup> <sup>2185</sup> <sup>2190</sup> <sup>2195</sup> <sup>2200</sup> <sup>2205</sup> <sup>2210</sup> <sup>2215</sup> <sup>2220</sup> <sup>2225</sup> <sup>2230</sup> <sup>2235</sup> <sup>2240</sup> <sup>2245</sup> <sup>2250</sup> <sup>2255</sup> <sup>2260</sup> <sup>2265</sup> <sup>2270</sup> <sup>2275</sup> <sup>2280</sup> <sup>2285</sup> <sup>2290</sup> <sup>2295</sup> <sup>2300</sup> <sup>2305</sup> <sup>2310</sup> <sup>2315</sup> <sup>2320</sup> <sup>2325</sup> <sup>2330</sup> <sup>2335</sup> <sup>2340</sup> <sup>2345</sup> <sup>2350</sup> <sup>2355</sup> <sup>2360</sup> <sup>2365</sup> <sup>2370</sup> <sup>2375</sup> <sup>2380</sup> <sup>2385</sup> <sup>2390</sup> <sup>2395</sup> <sup>2400</sup> <sup>2405</sup> <sup>2410</sup> <sup>2415</sup> <sup>2420</sup> <sup>2425</sup> <sup>2430</sup> <sup>2435</sup> <sup>2440</sup> <sup>2445</sup> <sup>2450</sup> <sup>2455</sup> <sup>2460</sup> <sup>2465</sup> <sup>2470</sup> <sup>2475</sup> <sup>2480</sup> <sup>2485</sup> <sup>2490</sup> <sup>2495</sup> <sup>2500</sup> <sup>2505</sup> <sup>2510</sup> <sup>2515</sup> <sup>2520</sup> <sup>2525</sup> <sup>2530</sup> <sup>2535</sup> <sup>2540</sup> <sup>2545</sup> <sup>2550</sup> <sup>2555</sup> <sup>2560</sup> <sup>2565</sup> <sup>2570</sup> <sup>2575</sup> <sup>2580</sup> <sup>2585</sup> <sup>2590</sup> <sup>2595</sup> <sup>2600</sup> <sup>2605</sup> <sup>2610</sup> <sup>2615</sup> <sup>2620</sup> <sup>2625</sup> <sup>2630</sup> <sup>2635</sup> <sup>2640</sup> <sup>2645</sup> <sup>2650</sup> <sup>2655</sup> <sup>2660</sup> <sup>2665</sup> <sup>2670</sup> <sup>2675</sup> <sup>2680</sup> <sup>2685</sup> <sup>2690</sup> <sup>2695</sup> <sup>2700</sup> <sup>2705</sup> <sup>2710</sup> <sup>2715</sup> <sup>2720</sup> <sup>2725</sup> <sup>2730</sup> <sup>2735</sup> <sup>2740</sup> <sup>2745</sup> <sup>2750</sup> <sup>2755</sup> <sup>2760</sup> <sup>2765</sup> <sup>2770</sup> <sup>2775</sup> <sup>2780</sup> <sup>2785</sup> <sup>2790</sup> <sup>2795</sup> <sup>2800</sup> <sup>2805</sup> <sup>2810</sup> <sup>2815</sup> <sup>2820</sup> <sup>2825</sup> <sup>2830</sup> <sup>2835</sup> <sup>2840</sup> <sup>2845</sup> <sup>2850</sup> <sup>2855</sup> <sup>2860</sup> <sup>2865</sup> <sup>2870</sup> <sup>2875</sup> <sup>2880</sup> <sup>2885</sup> <sup>2890</sup> <sup>2895</sup> <sup>2900</sup> <sup>2905</sup> <sup>2910</sup> <sup>2915</sup> <sup>2920</sup> <sup>2925</sup> <sup>2930</sup> <sup>2935</sup> <sup>2940</sup> <sup>2945</sup> <sup>2950</sup> <sup>2955</sup> <sup>2960</sup> <sup>2965</sup> <sup>2970</sup> <sup>2975</sup> <sup>2980</sup> <sup>2985</sup> <sup>2990</sup> <sup>2995</sup> <sup>3000</sup> <sup>3005</sup> <sup>3010</sup> <sup>3015</sup> <sup>3020</sup> <sup>3025</sup> <sup>3030</sup> <sup>3035</sup> <sup>3040</sup> <sup>3045</sup> <sup>3050</sup> <sup>3055</sup> <sup>3060</sup> <sup>3065</sup> <sup>3070</sup> <sup>3075</sup> <sup>3080</sup> <sup>3085</sup> <sup>3090</sup> <sup>3095</sup> <sup>3100</sup> <sup>3105</sup> <sup>3110</sup> <sup>3115</sup> <sup>3120</sup> <sup>3125</sup> <sup>3130</sup> <sup>3135</sup> <sup>3140</sup> <sup>3145</sup> <sup>3150</sup> <sup>3155</sup> <sup>3160</sup> <sup>3165</sup> <sup>3170</sup> <sup>3175</sup> <sup>3180</sup> <sup>3185</sup> <sup>3190</sup> <sup>3195</sup> <sup>3200</sup> <sup>3205</sup> <sup>3210</sup> <sup>3215</sup> <sup>3220</sup> <sup>3225</sup> <sup>3230</sup> <sup>3235</sup> <sup>3240</sup> <sup>3245</sup> <sup>3250</sup> <sup>3255</sup> <sup>3260</sup> <sup>3265</sup> <sup>3270</sup> <sup>3275</sup> <sup>3280</sup> <sup>3285</sup> <sup>3290</sup> <sup>3295</sup> <sup>3300</sup> <sup>3305</sup> <sup>3310</sup> <sup>3315</sup> <sup>3320</sup> <sup>3325</sup> <sup>3330</sup> <sup>3335</sup> <sup>3340</sup> <sup>3345</sup> <sup>3350</sup> <sup>3355</sup> <sup>3360</sup> <sup>3365</sup> <sup>3370</sup> <sup>3375</sup> <sup>3380</sup> <sup>3385</sup> <sup>3390</sup> <sup>3395</sup> <sup>3400</sup> <sup>3405</sup> <sup>3410</sup> <sup>3415</sup> <sup>3420</sup> <sup>3425</sup> <sup>3430</sup> <sup>3435</sup> <sup>3440</sup> <sup>3445</sup> <sup>3450</sup> <sup>3455</sup> <sup>3460</sup> <sup>3465</sup> <sup>3470</sup> <sup>3475</sup> <sup>3480</sup> <sup>3485</sup> <sup>3490</sup> <sup>3495</sup> <sup>3500</sup> <sup>3505</sup> <sup>3510</sup> <sup>3515</sup> <sup>3520</sup> <sup>3525</sup> <sup>3530</sup> <sup>3535</sup> <sup>3540</sup> <sup>3545</sup> <sup>3550</sup> <sup>3555</sup> <sup>3560</sup> <sup>3565</sup> <sup>3570</sup> <sup>3575</sup> <sup>3580</sup> <sup>3585</sup> <sup>3590</sup> <sup>3595</sup> <sup>3600</sup> <sup>3605</sup> <sup>3610</sup> <sup>3615</sup> <sup>3620</sup> <sup>3625</sup> <sup>3630</sup> <sup>3635</sup> <sup>3640</sup> <sup>3645</sup> <sup>3650</sup> <sup>3655</sup> <sup>3660</sup> <sup>3665</sup> <sup>3670</sup> <sup>3675</sup> <sup>3680</sup> <sup>3685</sup> <sup>3690</sup> <sup>3695</sup> <sup>3700</sup> <sup>3705</sup> <sup>3710</sup> <sup>3715</sup> <sup>3720</sup> <sup>3725</sup> <sup>3730</sup> <sup>3735</sup> <sup>3740</sup> <sup>3745</sup> <sup>3750</sup> <sup>3755</sup> <sup>3760</sup> <sup>3765</sup> <sup>3770</sup> <sup>3775</sup> <sup>3780</sup> <sup>3785</sup> <sup>3790</sup> <sup>3795</sup> <sup>3800</sup> <sup>3805</sup> <sup>3810</sup> <sup>3815</sup> <sup>3820</sup> <sup>3825</sup> <sup>3830</sup> <sup>3835</sup> <sup>3840</sup> <sup>3845</sup> <sup>3850</sup> <sup>3855</sup> <sup>3860</sup> <sup>3865</sup> <sup>3870</sup> <sup>3875</sup> <sup>3880</sup> <sup>3885</sup> <sup>3890</sup> <sup>3895</sup> <sup>3900</sup> <sup>3905</sup> <sup>3910</sup> <sup>3915</sup> <sup>3920</sup> <sup>3925</sup> <sup>3930</sup> <sup>3935</sup> <sup>3940</sup> <sup>3945</sup> <sup>3950</sup> <sup>3955</sup> <sup>3960</sup> <sup>3965</sup> <sup>3970</sup> <sup>3975</sup> <sup>3980</sup> <sup>3985</sup> <sup>3990</sup> <sup>3995</sup> <sup>4000</sup> <sup>4005</sup> <sup>4010</sup> <sup>4015</sup> <sup>4020</sup> <sup>4025</sup> <sup>4030</sup> <sup>4035</sup> <sup>4040</sup> <sup>4045</sup> <sup>4050</sup> <sup>4055</sup> <sup>4060</sup> <sup>4065</sup> <sup>4070</sup> <sup>4075</sup> <sup>4080</sup> <sup>4085</sup> <sup>4090</sup> <sup>4095</sup> <sup>4100</sup> <sup>4105</sup> <sup>4110</sup> <sup>4115</sup> <sup>4120</sup> <sup>4125</sup> <sup>4130</sup> <sup>4135</sup> <sup>4140</sup> <sup>4145</sup> <sup>4150</sup> <sup>4155</sup> <sup>4160</sup> <sup>4165</sup> <sup>4170</sup> <sup>4175</sup> <sup>4180</sup> <sup>4185</sup> <sup>4190</sup> <sup>4195</sup> <sup>4200</sup> <sup>4205</sup> <sup>4210</sup> <sup>4215</sup> <sup>4220</sup> <sup>4225</sup> <sup>4230</sup> <sup>4235</sup> <sup>4240</sup> <sup>4245</sup> <sup>4250</sup> <sup>4255</sup> <sup>4260</sup> <sup>4265</sup> <sup>4270</sup> <sup>4275</sup> <sup>4280</sup> <sup>4285</sup> <sup>4290</sup> <sup>4295</sup> <sup>4300</sup> <sup>4305</sup> <sup>4310</sup> <sup>4315</sup> <sup>4320</sup> <sup>4325</sup> <sup>4330</sup> <sup>4335</sup> <sup>4340</sup> <sup>4345</sup> <sup>4350</sup> <sup>4355</sup> <sup>4360</sup> <sup>4365</sup> <sup>4370</sup> <sup>4375</sup> <sup>4380</sup> <sup>4385</sup> <sup>4390</sup> <sup>4395</sup> <sup>4400</sup> <sup>4405</sup> <sup>4410</sup> <sup>4415</sup> <sup>4420</sup> <sup>4425</sup> <sup>4430</sup> <sup>4435</sup> <sup>4440</sup> <sup>4445</sup> <sup>4450</sup> <sup>4455</sup> <sup>4460</sup> <sup>4465</sup> <sup>4470</sup> <sup>4475</sup> <sup>4480</sup> <sup>4485</sup> <sup>4490</sup> <sup>4495</sup> <sup>4500</sup> <sup>4505</sup> <sup>4510</sup> <sup>4515</sup> <sup>4520</sup> <sup>4525</sup> <sup>4530</sup> <sup>4535</sup> <sup>4540</sup> <sup>4545</sup> <sup>4550</sup> <sup>4555</sup> <sup>4560</sup> <sup>4565</sup> <sup>4570</sup> <sup>4575</sup> <sup>4580</sup> <sup>4585</sup> <sup>4590</sup> <sup>4595</sup> <sup>4600</sup> <sup>4605</sup> <sup>4610</sup> <sup>4615</sup> <sup>4620</sup> <sup>4625</sup> <sup>4630</sup> <sup>4635</sup> <sup>4640</sup> <sup>4645</sup> <sup>4650</sup> <sup>4655</sup> <sup>4660</sup> <sup>4665</sup> <sup>4670</sup> <sup>4675</sup> <sup>4680</sup> <sup>4685</sup> <sup>4690</sup> <sup>4695</sup> <sup>4700</sup> <sup>4705</sup> <sup>4710</sup> <sup>4715</sup> <sup>4720</sup> <sup>4725</sup> <sup>4730</sup> <sup>4735</sup> <sup>4740</sup> <sup>4745</sup> <sup>4750</sup> <sup>4755</sup> <sup>4760</sup> <sup>4765</sup> <sup>4770</sup> <sup>4775</sup> <sup>4780</sup> <sup>4785</sup> <sup>4790</sup> <sup>4795</sup> <sup>4800</sup> <sup>4805</sup> <sup>4810</sup> <sup>4815</sup> <sup>4820</sup> <sup>4825</sup> <sup>4830</sup> <sup>4835</sup> <sup>4840</sup> <sup>4845</sup> <sup>4850</sup> <sup>4855</sup> <sup>4860</sup> <sup>4865</sup> <sup>4870</sup> <sup>4875</sup> <sup>4880</sup> <sup>4885</sup> <sup>4890</sup> <sup>4895</sup> <sup>4900</sup> <sup>4905</sup> <sup>4910</sup> <sup>4915</sup> <sup>4920</sup> <sup>4925</sup> <sup>4930</sup> <sup>4935</sup> <sup>4940</sup> <sup>4945</sup> <sup>4950</sup> <sup>4955</sup> <sup>4960</sup> <sup>4965</sup> <sup>4970</sup> <sup>4975</sup> <sup>4980</sup> <sup>4985</sup> <sup>4990</sup> <sup>4995</sup> <sup>5000</sup> <sup>5005</sup> <sup>5010</sup> <sup>5015</sup> <sup>5020</sup> <sup>5025</sup> <sup>5030</sup> <sup>5035</sup> <sup>5040</sup> <sup>5045</sup> <sup>5050</sup> <sup>5055</sup> <sup>5060</sup> <sup>5065</sup> <sup>5070</sup> <sup>5075</sup> <sup>5080</sup> <sup>5085</sup> <sup>5090</sup> <sup>5095</sup> <sup>5100</sup> <sup>5105</sup> <sup>5110</sup> <sup>5115</sup> <sup>5120</sup> <sup>5125</sup> <sup>5130</sup> <sup>5135</sup> <sup>5140</sup> <sup>5145</sup> <sup>5150</sup> <sup>5155</sup> <sup>5160</sup> <sup>5165</sup> <sup>5170</sup> <sup>5175</sup> <sup>5180</sup> <sup>5185</sup> <sup>5190</sup> <sup>5195</sup> <sup>5200</sup> <sup>5205</sup> <sup>5210</sup> <sup>5215</sup> <sup>5220</sup> <sup>5225</sup> <sup>5230</sup> <sup>5235</sup> <sup>5240</sup> <sup>5245</sup> <sup>5250</sup> <sup>5255</sup> <sup>5260</sup> <sup>5265</sup> <sup>5270</sup> <sup>5275</sup> <sup>5280</sup> <sup>5285</sup> <sup>5290</sup> <sup>5295</sup> <sup>5300</sup> <sup>5305</sup> <sup>5310</sup> <sup>5315</sup> <sup>5320</sup> <sup>5325</sup> <sup>5330</sup> <sup>5335</sup> <sup>5340</sup> <sup>5345</sup> <sup>5350</sup> <sup>5355</sup> <sup>5360</sup> <sup>5365</sup> <sup>5370</sup> <sup>5375</sup> <sup>5380</sup> <sup>5385</sup> <sup>5390</sup> <sup>5395</sup> <sup>5400</sup> <sup>5405</sup> <sup>5410</sup> <sup>5415</sup> <sup>5420</sup> <sup>5425</sup> <sup>5430</sup> <sup>5435</sup> <sup>5440</sup> <sup>5445</sup> <sup>5450</sup> <sup>5455</sup> <sup>5460</sup> <sup>5465</sup> <sup>5470</sup> <sup>5475</sup> <sup>5480</sup> <sup>5485</sup> <sup>5490</sup> <sup>5495</sup> <sup>5500</sup> <sup>5505</sup> <sup>5510</sup> <sup>5515</sup> <sup>5520</sup> <sup>5525</sup> <sup>5530</sup> <sup>5535</sup> <sup>5540</sup> <sup>5545</sup> <sup>5550</sup> <sup>5555</sup> <sup>5560</sup> <sup>5565</sup> <sup>5570</sup> <sup>5575</sup> <sup>5580</sup> <sup>5585</sup> <sup>5590</sup> <sup

Table IV—Continued

| Catalyst system and amount, ester exchange catalyst/polymerization catalyst (amount [part]) | Intrinsic viscosity [ $\zeta$ ] | Amount of residual carboxyl radicals (eq./ $10^6$ g) | Half crystallization time | Spinning temperature (°C) | Fineness (denier) | Yield strength (g/d) | Tenacity (g/d) | Elongation (%) | Young's Modulus (g/d) |
|---------------------------------------------------------------------------------------------|---------------------------------|------------------------------------------------------|---------------------------|---------------------------|-------------------|----------------------|----------------|----------------|-----------------------|
| Mn acetate/germanium dioxide (0.03 part/0.01 part)                                          | 0.79                            | 10                                                   | 3'40"                     | 300                       | 2.0               | 1.4                  | 3.4            | 57             | 105.6                 |
| Mn acetate/antimony trioxide (0.03 part/0.03 part)                                          | 0.78                            | 11                                                   | 4'30"                     | "                         | 2.0               | 1.4                  | 3.5            | 56             | 107.2                 |

## EXAMPLE 5

The polymer used in Example 1 was melt-extruded from a spinneret having holes of 2 mm length and various diameters, at a spinning temperature of 290°C.

Fibers whose monofilament denier was 2 were obtained at a take-up speed of 3000 m/min. The spinning conditions in this case are shown in the following Table V, in term of number of times of breakages of fibers in case of continuous spinning carried out for 8 hours. The physical properties of fibers obtained in the spinning carried out under the same conditions and by the use of a spinneret having holes of various lengths and diameters, are shown in Table VI, expressed in term of deviations from the arithmetic mean values in the measurements of 50 times.

Table V

| Hole diameter of spinneret (mm $\phi$ ) | Number of breakage of fibers (times) | 35 |
|-----------------------------------------|--------------------------------------|----|
| 0.15                                    | 5.6                                  | 40 |
| 0.2                                     | 3.1                                  |    |
| 0.25                                    | 0.9                                  |    |
| 0.3                                     | 0.5                                  |    |
| 0.4                                     | 0.4                                  |    |
| 0.5                                     | 0.5                                  |    |
| 0.7                                     | 0.4                                  | 45 |
| 0.9                                     | 0.6                                  |    |
| 1.0                                     | 1.7                                  |    |
| 1.2                                     | 2.9                                  |    |

Table VI

| Spinneret diameter (mm $\phi$ ) | Unevenness of denier ( $\pm$ denier) | Unevenness of tenacity ( $\pm$ g/d) | Unevenness of elongation ( $\pm$ %) | 50 |
|---------------------------------|--------------------------------------|-------------------------------------|-------------------------------------|----|
| 0.35                            | 1.0                                  | 0.2                                 | 1.5                                 | 13 |
|                                 | 1.5                                  | 0.1                                 | 1.0                                 | 7  |
|                                 | 2.0                                  | 0.15                                | 0.6                                 | 6  |
|                                 | 3.0                                  | 0.1                                 | 0.7                                 | 5  |
|                                 | 5.0                                  | 0.2                                 | 0.3                                 | 5  |
|                                 | 1.0                                  | 0.2                                 | 1.5                                 | 14 |
| 0.5                             | 2.0                                  | 0.2                                 | 0.9                                 | 8  |
|                                 | 3.0                                  | 0.15                                | 0.9                                 | 6  |
|                                 | 5.0                                  | 0.2                                 | 0.4                                 | 5  |
|                                 | 1.0                                  | 0.2                                 | 2.3                                 | 21 |
|                                 | 2.0                                  | 0.2                                 | 2.0                                 | 7  |
| 0.7                             | 2.0                                  | 0.1                                 | 0.9                                 | 6  |
|                                 | 5.0                                  | 0.15                                | 0.6                                 | 5  |
|                                 | 9.0                                  | 0.2                                 | 0.5                                 | 4  |
|                                 | 13.0                                 | 0.15                                | 0.5                                 | 5  |
|                                 |                                      |                                     |                                     | 55 |

## EXAMPLE 6

The polymer used in Example 1 was melt-extruded from a spinneret having a diameter of each hole of 0.35 mm $\phi$  and a length of 2 mm, at a temperature of 290°C. The temperature at the zone apart from the spinneret by 5 to 90 cm was maintained at a pre-determined point by installing a heating or cooling tube of 1 m length immediately below the spinneret. In another case, a cooling wind of -10°C was directly blown to the spinneret from a compressor. The physical properties of fibers whose monofilament denier was 2 and which were taken up at a take-up speed of 3000 m/min. in the above-mentioned cases, are shown in Table VII.

Table VII

| Temperature of atmosphere (°C) | 35 | Yield strength (g/d) | Tenacity (g/d) | Elongation (%) | Young's modulus (g/d) |
|--------------------------------|----|----------------------|----------------|----------------|-----------------------|
| -10°C                          |    | 0.7                  | 3.0            | 68             | 99.0                  |
| +5                             |    | 0.9                  | 3.0            | 63             | 102.1                 |
| 10                             |    | 1.3                  | 3.1            | 56             | 105.6                 |
| 20                             |    | 1.7                  | 3.4            | 51             | 110.0                 |
| 80                             |    | 1.8                  | 3.5            | 47             | 113.5                 |
| 100                            |    | 2.0                  | 3.6            | 43             | 116.3                 |
| 160                            |    | 2.1                  | 3.5            | 46             | 115.0                 |
| 180                            |    | 1.8                  | 3.4            | 50             | 113.6                 |
| 200                            |    | 0.9                  | 3.2            | 64             | 101.0                 |
| -10                            |    | 0.6                  | 3.0            | 69             | 93.6                  |
| (a cooling wind was blown)     |    |                      |                |                |                       |

A zone apart from the spinneret by more than 5 cm was maintained at 140°C by installing a heating tube of some length immediately below the spinneret. The spinning was carried out under the same condition as in the above-mentioned case. The physical properties of fibers of 2 denier are shown in Table VIII.

Table VIII

| 60 | Length of heating zone (cm) | Yield strength (g/d) | Tenacity (g/d) | Elongation (%) | Young's modulus (g/d) |
|----|-----------------------------|----------------------|----------------|----------------|-----------------------|
|    | 25                          | 0.8                  | 3.0            | 62             | 96.4                  |
|    | 30                          | 1.5                  | 3.2            | 50             | 107.3                 |
|    | 100                         | 2.0                  | 3.5            | 45             | 115.0                 |
|    | 200                         | 1.9                  | 3.4            | 46             | 116.3                 |
|    | 250                         | 2.1                  | 3.5            | 43             | 115.0                 |

## EXAMPLE 7

90 parts of 1,2-bis-p-carbomethoxyphenoxyethane and 7.5 parts of ethylene glycol were heated at 220°C, for 4 hours, in the presence of 0.04 part of barium acetate as an ester exchange catalyst, and formed methanol was eliminated. Thereafter, the resultant mixture was heated at 280°C, under a reduced pressure below 1 mm Hg, in a polymerization vessel, in the presence of a mixture of 0.03 part of dibutyl tin oxide as a polymerization catalyst and 0.03 part of TiO<sub>2</sub> as a delustering agent and 0.1 part of triphenyl phosphite as a stabilizer, and formed ethylene glycol was eliminated. The polymer thus obtained had an intrinsic viscosity of polymer of 0.73 and a residual carboxyl radical of polymer of 12 eq./10<sup>6</sup> g.

The polymer was melt-extruded from a spinneret having a diameter of each hole of 0.5 mmφ and a length of 3 mm, at a spinning temperature of 295°C, and resultant filaments were taken up at a take-up speed of 3000 m/min., while passing through a heating tube of 1 m length installed below the spinneret and maintained at 160°C. The fibers thus obtained whose monofilaments denier was 2 denier had a yield strength of 2.4 g/d., a tenacity of 4.2 g/d., an elongation of 38%, and a Young's modulus of 118 g/d., and were excellent in uniformity. In one Tan (a roll of cloth in Japanese unit, corresponding to about 12 yards) of plain fabric woven using these fibers, there were observed no dyeing unevenness.

What is claimed is:

1. A process for the direct spinning of commercial useful polyethylene-1,2-diphenoxymethane-p,p'-dicarboxylate fiber without any subsequent stretching operation which comprises extruding a melt of a polymer containing substantially 100 mol % of repetition units of the formula:



45

50

55

60

said polymer having an intrinsic viscosity of between about 0.4 and 1.3, and containing less than about 20.0 eq./10<sup>6</sup> g. of residual carboxyl group in the polymer, and taking up the resultant extruded fibers at a velocity ranging from about 1800 to 3500 m/min.

5 2. A process according to claim 1 wherein the melt of polyethylene-1,2-diphenoxymethane-p,p'-dicarboxylate is extruded through a spinneret having hole diameters within the range of 0.25 mm to 0.9 mm and a hole length within the range of 1.5 mm to 10 mm.

10 3. A process according to claim 1 wherein the extruded polyethylene-1,2-diphenoxymethane-p,p'-dicarboxylate is taken up after travelling through a zone maintained at 10°-180°C and which extends from the spinneret for at least 30 cm.

15 4. A process according to claim 1 wherein the fibers so produced have a yield strength of at least 1.0 g/d., an initial modulus of elasticity of at least 70 g/d., a breaking strength of at least 3.0 g/d., and a residual elongation of less than 80%.

20 5. The process according to claim 1 wherein said polymer is produced by subjecting 1,2-bis-(paracarbomethoxy)-phenoxyethane or its ester forming derivatives and ethylene glycol to ester-exchange reaction in the presence of a catalyst to form bisglycol of 1,2-bis-(paracarbomethoxy)-phenoxyethane and then subjecting the latter to condensation polymerization in the presence of a polymerization catalyst at an elevated temperature and under a reduced pressure while eliminating excessive glycol produced in the condensation.

\* \* \* \* \*

55

65